

April 27, 1926.

1,582,416

J. H. MASON

COATED FABRIC AND METHOD OF MAKING SAME

Original Filed April 14, 1920

Fig. 1.



Fig. 2.



INVENTOR  
*Jesse H. Mason*  
BY  
*Chester H. Russell, Jr.*  
ATTORNEY

## UNITED STATES PATENT OFFICE.

JESSE H. MASON, OF ROSELLE, NEW JERSEY, ASSIGNOR TO DURATEX CORPORATION, OF NEWARK, NEW JERSEY, A CORPORATION OF NEW JERSEY.

## COATED FABRIC AND METHOD OF MAKING SAME.

Application filed April 14, 1920, Serial No. 373,956. Renewed October 6, 1925.

To all whom it may concern:

Be it known that I, JESSE H. MASON, a citizen of the United States, residing at Roselle, New Jersey, have invented certain new and useful Improvements in Coated Fabrics and Methods of Making Same, of which I declare the following to be a full, clear, and exact description.

This invention relates to improvements in coated fabrics and the method of making same. This invention relates more particularly to rubber-coated fabrics in which an ornamental effect is produced by embossing the rubber-coated fabric.

Heretofore, it has been impossible to produce a two-color or two-tone effect in rubber-coated fabrics except by printing on the rubber-coated fabric any desired design in which one or more colors might be used. This method has been and is objectionable because the design thus produced on the coated fabric has a flat appearance and looks cheap. The product made in this manner, therefore, does not appeal to the buying public as a high grade material and it has not been possible in this manner to simulate the effect produced on real leather. As a rule the colored design thus printed on the coated fabric has a tendency to rub off.

One of the objects of my invention is to provide a new type of coated-fabric in which an ornamental effect is produced in more than one tone or color, giving a rich and pleasing appearance to the product.

Another object of my invention is to provide a rubber-coated fabric which is finished in more than one tone or color so as to simulate the multi-color effect produced in finishing natural leather.

Another object of my invention is to provide an improved process for producing a multi-color effect in rubber-coated fabrics.

In Fig. 1 of the drawing there is illustrated a section through fabric coated in accordance with the processes indicated in the application, and

Fig. 2 is a section through a base fabric having a modified formation.

In general, I accomplish the objects of my invention and avoid the objectionable features of prior methods which have been indicated above, by coating a fabric backing

with a base coat of rubber, embossing the base coat, and applying a surface coating carrying pigment, which may be of a different color from the base coat, so that the surface coating lodges in the crevices formed in the base coat by the embossing operation, but is rubbed off of the high spots of the base coat. The coated fabric produced in accordance with my invention, in general, comprises a fabric backing having a base coat of rubber with crevices therein in which a surface coating carrying pigment, which may be of a different color from the base coat, is lodged.

In carrying out my invention, I first apply to a suitable fabric backing, such as a drill, sateen or moleskin, a base coat of rubber composition. This rubber composition may be any satisfactory rubberizing compound. The particular formula does not form a part of my invention, appropriate formulæ being well known to those skilled in the rubber art, it being understood that the ingredients will vary depending upon the character, quality and color of the coating to be produced. This rubber compound may be applied to the backing on a calender or spreading machine in the manner well understood in the rubber art.

After the base coat is applied to the backing, it is embossed in the usual manner, either by passing the rubber-coated fabric between embossing rolls or by impressing the desired design on the base coat by embossing plates in a press.

After the embossing operation, a "soup" coat or "rub" is applied as will be described hereinafter. This "rub" comprises a suitable carrier containing pigment or dye to give color to the "rub". The pigment used may be such as to give the "rub" a different color from the base coat so that the multi-color effect may be produced by the contrast between the color of the "rub" and that of the base coat, as will appear more clearly hereinafter. I have secured very desirable results by the use of two different carriers for the pigment, both of which I will describe, it being understood that either of these carriers may be employed. I may use as a carrier for the pigment in the "rub" coat a vulcanizing varnish made up of a vegetable

drying oil and sulphur. For instance, I may make up a "rub" coat by adding about eight pounds of sulphur to about twenty-five, 5 gallons of boiled linseed oil and add to this the pigments or dyes necessary to give the "rub" coat the desired color. These ingredients are intimately mixed and the mixture thinned down until it is of the proper consistency for application to the base coat. 10 Instead of the "rub" coat described above, I may use one in which rubber cement is used as the carrier for the pigment. For instance, I may dissolve rubber in a suitable rubber solvent, add the sulphur necessary 15 for vulcanization and the pigments or dyes necessary to give the desired color to the "rub" coat. These ingredients are intimately mixed, brought to the proper consistency, and applied to the base coat in the manner 20 which I will describe.

The "rub" coat is applied to the base coat by drawing the fabric carrying the embossed rubber base coat beneath a spreading knife while the fluid "rub" coat is fed in front of 25 the spreading knife. This method of applying a coating is well known in the art and needs no further description to be understood by those familiar with this art. The tension of the fabric and the rate of feed of the "rub" 30 coat in front of the knife is regulated and adjusted so that the "rub" coat lodges in the crevices formed in the base coat by the embossing operation and is rubbed off of the high spots by the spreading knife so 35 that the base coat is exposed at the high spots.

After the application of the "rub" coat, I may, when desired, apply a transparent 40 top coat of a clear vulcanizing varnish. For instance, I add about eight pounds of sulphur to about twenty-five gallons of boiled linseed oil, mix these ingredients intimately, thin to the proper consistency and apply by a spreading knife. I use a transparent 45 top coat in cases where the pigments are of such nature that the finished product would otherwise be likely to crock or rub off.

The material coated as described above is then fed in the heater where it is cured 50 or vulcanized by exposure to heat in the manner well known in the art. The curing operation may follow directly after the application of the "rub" coat or, in cases where 55 a top coat is applied, it may follow the application of the top coat.

It will appear that the material produced in accordance with the process which I have described is characterized by a base coat of rubber having crevices or depressions in 60 which a suitable vulcanizing carrier carrying pigment is deposited, the pigment being of a different or contrasting color from the color of the base coat, so that a two-color or two-tone effect is obtained in this way. 65 Since the final step in the process is the

vulcanizing of all of the materials deposited on the backing, they are all amalgamated into a single compact mass so that the pigments will not crock or rub off. This is particularly true where they are covered by 70 a top coat as described.

I am aware that the particular embodiment of my invention, which I have described here, is susceptible of considerable variation without departing from the spirit 75 of my invention and, therefore, I desire to claim the same broadly, as well as specifically, as indicated by the appended claims.

Having thus described my invention, what I claim as new and desire to secure by 80 Letters Patent is:

1. The process of making coated fabrics comprising applying a base coat of rubber composition to a suitable backing, forming elevations and depressions in the base coat, 85 and depositing a coating carrying coloring matter in the depressions of the base coat while leaving the elevations substantially uncoated.

2. The process of making coated fabrics comprising applying a base coat of rubber composition to a suitable backing, forming elevations and depressions in said base coat, depositing a coating carrying coloring matter in the depressions formed in the base 95 coat, and then vulcanizing the coated material, said base coat being free from the coating exterior to said depressions.

3. The process of making coated fabrics comprising applying a base coat of rubber composition to a suitable backing, forming elevations and depressions in said base coat, depositing a coating carrying coloring matter in the depressions only formed in 100 said base coat, applying a top coat, and vulcanizing the coated material. 105

4. The process of making coated fabrics comprising applying a base coat of rubber composition to a suitable backing, forming elevations and depressions in said base coat, and depositing a coating comprising a vulcanizable carrier and coloring matter in the 110 depressions formed in said base coat, and then vulcanizing the coated material, said base coat being free from the coating exterior to said depressions.

5. The process of making coated fabrics comprising applying a base coat of rubber composition to a suitable backing, forming elevations and depressions in said base coat, depositing a coating comprising a vulcanizable carrier and coloring matter in the 115 depressions formed in said base coat, thereby leaving the base coat exposed on the elevations, and then vulcanizing the coated material.

6. The process of making coated fabrics comprising applying a base coat of rubber composition to a suitable backing, forming elevations and depressions in the said base 120

- coat, depositing a coating comprising a vulcanizable carrier and coloring matter in the depressions formed in said base coat, applying a transparent top coat, and then vulcanizing the coated material, said base coat being free from the coating exterior to said depressions.
7. The process of making coated fabrics comprising applying a base coat of rubber composition to a suitable backing, forming elevations and depressions in the said base coat, depositing a coating comprising a vulcanizable carrier, sulphur and coloring matter in the depressions only formed in said base coat, and then vulcanizing the coated material.
8. The process of making coated fabrics comprising applying a base coat of rubber composition to a suitable backing, forming elevations and depressions in the said base coat, depositing a coating comprising a vulcanizing varnish like material and coloring matter in the depressions formed in the base coat while leaving the elevations uncoated, and then vulcanizing the coated material.
9. The process of making coated fabrics comprising applying a base coat of rubber composition to a suitable backing, forming elevations and depressions in the said base coat, depositing a coating comprising boiled linseed oil, sulphur and coloring matter in said depressions, and then vulcanizing the coated material, said base coat being free from the coating exterior to said depressions.
10. The process of making coated fabrics comprising applying a base coat of rubber composition to a suitable backing, forming elevations and depressions in the said base coat, depositing a coating comprising a varnish like material and coloring matter in the said depressions, then applying a top coat of vulcanizing varnish, and finally vulcanizing the coated material.
11. The process of making coated fabrics comprising applying a base coat of rubber composition to a suitable backing, embossing the base coat, depositing a coating comprising a sulphur containing varnish like material and coloring matter in the depressions formed in the base coat by the embossing, applying a top coat of vulcanizing varnish, and then vulcanizing the coated material.
12. The process of making coated fabrics comprising applying a base coat of rubber composition to a suitable backing, embossing the base coat, depositing a coating comprising boiled linseed oil, sulphur and coloring matter in the depressions only formed in the base coat by the embossing, applying a top coat, and then vulcanizing the coated material.
13. A coated fabric comprising a suitable backing, a base coat of rubber composition carried thereby and having depressions formed therein, a coating carrying suitable coloring matter deposited in said depressions only, and a transparent top coat, all of said coatings being vulcanized.
14. A coated fabric comprising a suitable backing, a base coat of rubber composition carried thereby and having depressions formed therein, and a coating carrying coloring matter deposited in said depressions and exposing the higher portions, said coatings being vulcanized as a unitary mass.
15. A coated fabric comprising a suitable backing, a base coat of rubber composition carried thereby and having depressions formed therein, and a vulcanized coating carrying coloring matter deposited in said depressions, said coatings being vulcanized as a unitary mass, said base coat being free from the coating exterior to said depressions.
16. A coated fabric comprising a suitable backing, a base coat of rubber composition carried thereby and having depressions formed therein, and a coating deposited in said depressions and comprising a vulcanized carrier, sulphur and coloring matter, said coatings being vulcanized as a unitary mass, said base coat being free from the coating exterior to said depressions.
17. A coated fabric comprising a suitable backing, a base coat of rubber composition carried thereby and having depressions formed therein, and a coating deposited in said depressions and comprising a varnish like material, and suitable coloring matter, said coatings being vulcanized as a unitary mass, said base coat being free from the coating exterior to said depressions.
18. A coated fabric comprising a suitable backing, a base coat of rubber composition carried thereby and having depressions formed therein, and a coating deposited in said depressions and comprising boiled linseed oil, sulphur and coloring matter, said coatings being vulcanized as a unitary mass, said base coat being free from the coating exterior to said depressions.
19. A coated fabric comprising a suitable backing, a base coat of rubber composition carried thereby and having depressions formed therein, a coating deposited in said depressions only and comprising varnish like material and suitable coloring matter carried thereby, and a transparent top coat, all of said coatings being vulcanized.
20. A coated fabric comprising a suitable backing, a base coat of rubber composition carried thereby and having depressions formed therein, and a coating carrying coloring matter lodged in said depressions and exposing the higher portions of said base coat.
21. A coated fabric comprising a suitable backing, a base coat of rubber composition carried thereby and having depressions formed therein, and a coating carrying suit-

able coloring matter deposited in said depressions while exposing the higher portions and vulcanized to said base coat.

22. The process of making coated fabrics comprising applying a base coat of rubber composition to a suitable backing, embossing the base coat, depositing a coating comprising a vegetable drying oil, sulphur and

coloring matter in the depressions formed in the base coat by the embossing, and then <sup>10</sup> vulcanizing the coated material, said base coat being free from the coating exterior to said depressions.

In testimony whereof, I affix my signature.

JESSE H. MASON.